

Sept. 3, 1935.

H. L. LEVIN

2,013,351

SIDING MATERIAL

Filed Oct. 12, 1931



INVENTOR.  
*Harold L. Levin*

BY *Samuel Stearns*  
ATTORNEY.

## UNITED STATES PATENT OFFICE

2,013,351

## SIDING MATERIAL

Harold L. Levin, Rutherford, N. J., assignor to  
The Patent and Licensing Corporation, Boston,  
Mass., a corporation of Massachusetts

Application October 12, 1931, Serial No. 568,259

1 Claim. (Cl. 20—5)

This invention relates to asphaltic composition siding material and to a method of producing it.

Siding strips as heretofore produced by severing strips from a sheet of fibrous felted material, 5 saturated and coated with waterproofing material and surfaced with granular material, such as crushed slate, have several objectionable characteristics. The exposed cut edges permit access of moisture to the interior of the strips causing 10 swelling and bulking with the result that the strips crack and curl. Furthermore, siding material made in this manner is comparatively light and thin in the proximity of its exposed edges and is not only unattractive but is easily bent by the 15 wind so that it does not lie flush against the side of the building.

When the siding is to be laid in such manner as to simulate bricks and mortar joints it is necessary to provide, between adjacent courses, a band 20 area of different color from the brick-simulating surface. Where this band is produced by a surfacing of granular material differing in color from that of the brick simulating surfaces it is difficult to obtain a straight and even line of demarcation between the differently colored areas necessary to produce the brick-simulating effect when the material is laid.

The object of my invention is to provide an asphaltic composition siding element constructed 30 to afford increased durability in service.

Another object is to provide a siding element of this character, designed to present, when laid in successive courses, an appearance simulating ordinary brick wall construction.

Still another object resides in the provision of a method for producing these elements in such a way as to insure the attainment of a straight line of demarcation between the differently colored zones which effect the brick-simulating appearance when the elements are laid.

A further object of the invention is to provide a very simple method of producing brick-simulating siding elements of the above described character, in a rapid and efficient manner.

The strips produced according to my invention are attractive and have superior weather-resisting qualities since the exposed surfaces and edges are covered by an additional coating which additionally protects these surfaces and seals the exposed edges against the deteriorating action of the weather. I have further made provision for additionally strengthening the strip at the points where they are fastened to the substructure.

Further advantages will manifest themselves

from the following description, in conjunction with the accompanying drawing of which,

Figure 1 illustrates the arrangement of a number of elements for the purpose of coating and surfacing the weather exposed portions;

Figure 2 represents several finished strips, having strengthened portions at the places where the strip is fastened to the substructure, as they appear when laid in place; and

Figure 3 is a side view similar to Figure 2, illustrating a modified form of siding strip.

Referring to Figure 1, the numerals 1 to 8 represent a plurality of strips arranged in overlapping relation for the purpose of coating and surfacing the exposed areas. These strips may be cut from a sheet of asphalt saturated and 15 coated flexible fibrous material which may be surfaced with granular material, preferably of fine mesh, or left unsurfaced. The elements as cut are substantially rectangular in shape, and have body portions 9 and rectangular tabs 10 extending therefrom separated by narrow cut-outs 11. The strips are arranged in an overlapping series with the side edges 12 and 13 coincident, and with the butt edges 14 extending a small distance below the upper edge 15 of the cut-outs 11 20 of the subjacent strip. The portion of the top-most element which is not to be coated may be blocked out by a suitable template. Asphalt or 25 similar waterproofing substance is then sprayed or filmed over the entire surface presented by 30 the series of overlapping elements and then covered with coarse granular material such as granulated slate or slag. The elements are separated in any desirable manner and subjected to pressure to firmly embed the granular material in the 35 asphalt.

The finished elements will have the major portion of the tabs 10 surfaced with coarse granular material of different color than the fine granular material on the body portion 9. The tongues 16 40 which are formed along the portions exposed by the cut-outs of the superjacent strip in the series will also be surfaced with coarse granular material of the same color and mesh as that on the tabs 10. The bottom and side edges 14, 17 and 18 of the 45 tabs and inner edges 15 of the notches will be coated with asphalt, thereby sealing them against access of moisture to the fibrous base and will also be surfaced with coarse granular material at the same time that the coating and surfacing is applied to the face of the tabs, thereby forming a continuous and integral coating over the surface and edges. If for any reason it is not desired to coat and surface the areas 16, they may be blocked 50 55

out in any suitable manner, as for example, by inserting a sheet of suitable material under each strip so as to underlie the cut-outs 11.

When laid in place on a wall or like surface, the 5 elements will be arranged as shown in Figure 2. The bottom edges 14 of the tabs will be coincident with the inner edges 15 of the cut-outs, thereby exposing horizontal bands 19 between adjacent courses, differing in color from that of the tabs. 10 These bands simulate horizontal mortar-joints. The body portions 20 exposed beneath the cut-outs are of the same color as the bands 19 and simulate the vertical mortar-joints. As is apparent from Figure 2, the adjacent courses are 15 staggered in relation to each other so that the cut-outs of the subjacent course occur intermediate the cut-outs of the superjacent course. The strips may be fastened by means of nails, staples, or the like as indicated at 21 in Fig. 2 driven 20 through the tongues 16. Since these portions have additional thickness by virtue of the extra layer of coating and granular material they afford strong points for fastening.

In Figure 3, I have illustrated the appearance 25 of several courses of siding elements embodying features of my invention, but formed without the tongues.

The butt portions of the elements have increased weight due to the secondary layers of 30 asphalt and coarse granular material and for that reason will lie in place much more effectively than elements in which the exposed portions are of comparatively thin structure. By applying the added weather protecting material only to those 35 portions of the strips where it is most required, a highly desirable product can be made at a comparatively low cost.

Other forms of siding elements, as for example, those resembling clapboard can be coated in a 40 similar manner. The strips may be overlapped so as to expose narrow bands along the lower margins which together with the exposed edges may be coated and surfaced preferably to con-

trast with the remainder of the exposed portion of the strips.

My invention is subject to various modifications. For example, the coating can be done with cold asphalt in the dispersed form. In lieu of asphalt saturated and coated felted fibrous material, mastic composed of a homogeneous mixture of asphalt, fibrous material and hardening fillers may be used as the base for making the preformed elements or blanks to be treated in accordance 10 with this invention. Moreover, the granular material used for initially surfacing the strip may be of the same size as that used for the secondary surfacing on the exposed portions. The tabs may be surfaced with granular material of varigated 15 color, and if desired, each tab on a strip may differ in color from the other tabs. The portion of the strip exposed as a horizontal band between successive courses as well as the portions exposed beneath the cut-outs may also be surfaced with granular material differing in color from the remaining portion of the strip or these portions may be coated with asphalt and left unsurfaced. Any or all of these modifications fall within the scope 20 of my invention.

I claim as my invention:

A siding element of asphaltic composition having a body portion and tabs spaced by narrow cut-outs extending from said body portion, a layer of asphaltic coating surfaced with granular material 30 covering substantially the entire upper surface of said element, an additional layer of asphaltic coating surfaced with coarse granular material differing in color from the first named granular material and covering the major portion of the exposed 35 face of said tabs from the butt edges to a line parallel to and below the upper ends of said cut-outs, said additional layer extending also around the exposed edges of the tabs, and similar additional layers of asphalt surfaced with similar coarse granular material extending in tongues up- 40 wardly from the upper ends of said cut-outs.

HAROLD L. LEVIN